

# United States Patent

Kasai et al.

[15] 3,690,062

[45] Sept. 12, 1972

[54] **HARD WATCH CASE**

[72] Inventors: **Masami Kasai, Yoshiaki Fujimori,**  
born of Nagano, Japan

[73] Assignee: **Kabashiki Kaisha Suwa, Seikosha**  
Tokyo, Japan

[22] Filed: **Jan. 29, 1971**

[21] Appl. No.: **110,960**

[30] **Foreign Application Priority Data**

Jan. 30, 1970 Japan .....45/7674

[52] U.S. Cl. .....58/88 R, 58/88 G

[51] Int. Cl. .....G04b 37/00

[58] Field of Search .....58/88, 90 R, 106.5; 117/129,  
117/135.1

[56] **References Cited**

UNITED STATES PATENTS

2,843,507 7/1958 Long .....117/129  
2,672,426 3/1954 Grubel et al. ....117/129 X

3,179,524 4/1965 Hunter.....117/129 X  
3,482,951 12/1969 Hubbell et al. ....117/129 X

FOREIGN PATENTS OR APPLICATIONS

3,079 3/1891 Switzerland .....58/88

Primary Examiner—Richard B. Wilkinson

Assistant Examiner—George H. Miller, Jr.

Attorney—Blum, Moscovitz, Friedman & Kaplan

[57] **ABSTRACT**

A watch case resistant to mechanical defacement and corrosion, having an external pressed and sintered component at least a part of which comprises at least one material selected from the group consisting of  $\text{Al}_2\text{O}_3$ ,  $\text{BeO}$ ,  $\text{CeO}_2$ ,  $\text{Cu}_2\text{O}$ ,  $\text{Cr}_2\text{O}_3$ ,  $\text{CoO}$ ,  $\text{Fe}_2\text{O}_3$ ,  $\text{Fe}_3\text{O}_4$ ,  $\text{MgO}$ ,  $\text{MnO}$ ,  $\text{NiO}$ ,  $\text{Nb}_2\text{O}_3$ ,  $\text{SiO}_2$ ,  $\text{Ta}_2\text{O}_5$ ,  $\text{ThO}_2$ ,  $\text{SnO}_2$ ,  $\text{TiO}_2$ ,  $\text{V}_2\text{O}_3$ ,  $\text{ZnO}$ ,  $\text{ZrO}_2$ ,  $\text{Al}_2\text{O}_3$ ,  $\text{SiO}_2$ ,  $\text{Al}_2\text{O}_3$ ,  $\text{TiO}_2$ ,  $\text{BeO}\cdot\text{Al}_2\text{B}(3)$ ,  $\text{CoO}\cdot\text{Al}_2\text{O}_3$ ,  $\text{MgO}\cdot\text{Al}_2\text{O}_3$ ,  $\text{MgO}\cdot\text{ZrO}_2\cdot\text{SiO}_2$ ,  $\text{ZnO}\cdot\text{Al}_2\text{B}(3)$  and  $\text{ZrO}_2\cdot\text{SiO}_2$ .

11 Claims, 4 Drawing Figures



PATENTED SEP 12 1972

3,690,062

FIG. 1



FIG. 2



FIG. 3



FIG. 4



## HARD WATCH CASE

## BACKGROUND OF THE INVENTION

In the mass production of conventional watch cases the materials which have been used principally are gold, gold alloy and stainless steel. All of these materials, however, have a low surface hardness (Vickers hardness, 200 maximum); as a result, they are easily scratched or otherwise defaced by contact with other hard metals or concrete. The high surface polish is lost relatively quickly during the wearing of the time-piece. Moreover, using the above-mentioned metals the case color is restricted either to those of gold or stainless steel. Furthermore, gold and its alloys have high specific gravities as is shown in Table I. In consequence, large watch cases can be sufficiently heavy to constitute an annoyance to the wearer. Also, gold and its alloys are expensive.

## SUMMARY OF THE INVENTION

We have found that a number of oxides which have hitherto been used for the manufacture of brick, board, crucibles, and refractory tools can be fashioned into parts of watch cases or entire watch cases which are mechanically strong, resistant to abrasion, and resistant to corrosion. Suitable oxides maybe the oxides of single metals such as  $Al_2O_3$ , or compounds as in the case of  $MgO \cdot Al_2O_3 \cdot 3$ . Also oxides may be used along or in combination. These oxides, when pressed and sintered, are very hard, resistant to corrosion and mechanical defacement and make available a choice of colors.

TABLE I

## Characteristics of Various Materials For a Watch Case

| Materials            | Specific Gravity (g/cc) | Hardness (Knoop) | Color       |
|----------------------|-------------------------|------------------|-------------|
| WC                   | 15.8                    | 1880             | Black       |
| $Al_2O_3$            | 3.9                     | 1930             | Pure White  |
| $ZrO_2$              | 5.4                     | (7)              | Yellow      |
| $MgO \cdot Al_2O_3$  | 3.3                     | (8)              | Colorless   |
| 18-8 Stainless Steel | 7.9                     | 200              | Transparent |
| Au                   | 19.3                    | 50               | Gray        |
|                      |                         |                  | Yellow      |

Note: FIGURES in ( ) shown Mohs hardness.

Table I also gives data for tungsten carbide and for stainless steel and for gold. As is evident from the table tungsten carbide and gold are much heavier than the representative oxides tabulated. While the carbide is hard as shown by the corresponding entry in the table, stainless steel and gold are soft.

It is an object of the invention to provide a watch case of improved hardness, durability, chemical stability and appearance.

It is a further object of the invention to provide a watch case of low weight.

It is another object of the invention is to provide a hard, durable, abrasion-resistant surface element of attractive appearance for watch cases of conventional materials.

Still other objects and advantages of the invention will in part be obvious and will in part be apparent from the specification.

## BRIEF DESCRIPTION OF THE DRAWINGS

FIG. 1 is a sectional view of a watch case in which a composition in accordance with the present invention is used as a surface protection;

FIG. 2 is a sectional view of a watch case in which a bezel of a composition in accordance with the present invention is used to protect the top surface of a case of conventional composition;

FIG. 3 is a sectional view of a watch case in which an element having a composition in accordance with the present invention is used to protect the upper and side surfaces of a watch case of conventional composition; and

FIG. 4 is a sectional view of a watch case, the entire body of which is made of a composition in accordance with the present invention.

## DESCRIPTION OF THE PREFERRED EMBODIMENTS

A mixture of powdered raw material having a particle size of 1-2 microns and consisting of 94 percent by weight of  $Al_2O_3$ , 3 percent by weight of  $SiO_2$ , 1 percent by weight of  $MgO$ , 0.5 percent by weight of  $TiO_2$ , and 1.5 percent by weight of  $Fe_2O_3$  is pulverized and mixed in a ball mill for about 100 hours. A lubricant, preferably of the paraffin group, is added to make the mixture suitable for pressing. The material is formed into the desired shape at a pressure of about 2 ton/cm<sup>2</sup>. The composition is then sintered for about an hour at a temperature of 1650° to 1750° C. The resultant product is extremely hard and is then diamond-polished. The product is sapphire blue in color and has a Vickers hardness of 1650 to 1730. As a result of this great hardness, the surface resists scratching by knife, razor, scissors, glass or file. In addition to being resistant to mechanical defacement, the material also shows excellent resistance to artificial sweat and sea water. The material can therefore be considered sufficiently resistant to corrosion to be suitable for use as a watch case. The specific gravity of the product is about 4.0 g/cc so that product cases are substantially lighter than conventional cases of stainless steel, gold, or gold alloy. Such cases are also lighter than cases made of carbide when sintered with heavy metal binders such as nickel, cobalt or molybdenum.

In another embodiment, powdered raw material having a particle size of 1-2 microns and consisting of 95 percent by weight of  $MgO \cdot Al_2O_3$ , 3.5 percent by weight of  $SiO_2$ , 0.5 percent of  $CoO$  and 1.0 percent of  $MnO$  is treated in a manner similar to that described above. The product of this example is also very hard and can be polished only with diamond. The product has a Vickers hardness of 1780 to 1860, its color is a beautiful blue, and its specific gravity is 3.8g/cc. It should be noted that this example differs from the previous example in that a compound oxide, namely  $MgO \cdot Al_2O_3$ , is used as the principal ingredient.

Materials which may be used alone or in combination are the simple oxides,  $Al_2O_3$ ,  $BeO$ ,  $CeO_2$ ,  $Cu_2O$ ,  $Cr_2O_3$ ,  $CoO$ ,  $Fe_2O_3$ ,  $Fe_3O_4$ ,  $MgO$ ,  $MnO$ ,  $NiO$ ,  $Nb_2O_3$ ,  $SiO_2$ ,  $Ta_2O_5$ ,  $ThO_2$ ,  $SnO_2$ ,  $TiO_2$ ,  $V_2O_3$ ,  $ZnO$  and  $ZrO_2$ , and the compound oxides  $Al_2O_3 \cdot SiO_2$ ,  $Al_2O_3 \cdot TiO_2$ ,  $BeO \cdot Al_2O_3$ ,  $CoO \cdot Al_2O_3$ ,  $MgO \cdot Al_2O_3$ ,  $MgO \cdot ZrO_2 \cdot SiO_2$ ,  $ZnO \cdot Al_2O_3$ , and  $ZrO_2 \cdot SiO_2$ . As the second example given above showed, a compound oxide may

be used in combination with simple oxides. Also, the strength of the product may be increased and the range of colors may be increased by adding one or more metals to the combination of the oxides and compound oxides examples of such metals are Ni, Co, and Mo. In particular, the hardness may be very substantially increased by adding boron to compositions.

In view of the great hardness and low deformability of compositions prepared in accordance with the present invention it is desirable that the design of the watch case take these properties into account. In FIG. 1, the hard layer 1 is superimposed on a case body 2 of stainless steel. The hard layer 1 is attached to the case body 2 by cementing. The case body, being of stainless steel, is easily fabricated and the upper surface of the case is protected from marring by the superimposed hard layer 1.

In FIG. 2 the protective layer 1 is in the form of a bezel covering most of the outer surface of the case body 2. The bezel is held to the body 2 by means of the snap-ring 3. Since the bezel is essentially non-deformable, deformability must be provided in the body; deformability of the body is provided by means of the groove 4 behind the snap-ring 3.

In the example of FIG. 3 the outer case body 1 and the lug 5 are composed of materials of the type described herein. The body 2 is made of stainless steel which, as mentioned above, is easily processed. Grooves 3 and 4 are cut into the peripheral portion of the inner case body and serve to permit insertion of a binding agent for holding the outer case to the inner case body.

FIG. 4 shows a watch case in which the entire body including the back cover is made of one of the hard materials described herein. In a watch case of this design, no part of the case can be scratched.

It will thus be seen that the objects set forth above, among those made apparent from the preceding description, are efficiently attained and, since certain changes may be made in the above composition of matter without departing from the spirit and scope of the invention, it is intended that all matter contained in the above description shall be interpreted as illustrative

and not in a limiting sense.

What is claimed is:

1. A watch case resistant to mechanical defacement and corrosion, having an external pressed and sintered component at least a part of which comprises at least one material selected from the group consisting of

Al<sub>2</sub>O<sub>3</sub>, BeO, CeO<sub>2</sub>, Cu<sub>2</sub>O, Cr<sub>2</sub>O<sub>3</sub>, CoO, Fe<sub>2</sub>O<sub>3</sub>, Fe<sub>3</sub>O<sub>4</sub>, MgO, MnO, NiO, Nb<sub>2</sub>O<sub>3</sub>, SiO<sub>2</sub>, Ta<sub>2</sub>O<sub>5</sub>, ThO<sub>2</sub>, SnO<sub>2</sub>, TiO<sub>2</sub>, V<sub>2</sub>O<sub>3</sub>, ZnO, ZrO<sub>2</sub>, Al<sub>2</sub>O<sub>3</sub> · SiO<sub>2</sub>, Al<sub>2</sub>O<sub>3</sub> · TiO<sub>2</sub>, BeO · Al<sub>2</sub>O<sub>3</sub>, CoO · Al<sub>2</sub>O<sub>3</sub>, MgO · Al<sub>2</sub>O<sub>3</sub>, MgO · ZrO<sub>2</sub> · SiO<sub>2</sub>, ZnO · Al<sub>2</sub>O<sub>3</sub> and ZrO<sub>2</sub> · SiO<sub>2</sub>.

15 2. A watch case as defined in claim 1 wherein said external component chiefly comprises the simple oxides listed in claim 1.

15 3. A watch case as defined in claim 1 wherein said external component chiefly comprises the compound oxides listed in claim 1.

20 4. A watch case as defined in claim 1 further comprising a metal selected from the group consisting of Ni, Co and Mo.

5. A watch case as defined in claim 1 further comprising boron.

25 6. A watch case as defined in claim 1 wherein said external component includes a case cover and a case body.

7. A watch case as defined in claim 6 wherein said case cover and case body are of one-piece construction.

30 8. A watch case as defined in claim 1 further comprising a stainless steel body, the outer portion of which is covered by said pressed and sintered external component.

9. A watch case as defined in claim 8 wherein said pressed and sintered external component is a bezel.

35 10. A watch case as defined in claim 8 wherein said external component is mechanically engaged with said stainless steel body.

40 11. A watch case as defined in claim 8 wherein said external component is cemented to said stainless steel body.

\* \* \* \* \*

UNITED STATES PATENT OFFICE  
CERTIFICATE OF CORRECTION

Patent No. 3,690,062 Dated Sept. 12, 1972

Inventor(s) Masami Kasai, Yoshiaki Fujimori

It is certified that error appears in the above-identified patent and that said Letters Patent are hereby corrected as shown below:

In the Abstract, line 8, "Al<sub>2</sub>B(3)" should read --Al<sub>2</sub>O<sub>3</sub>--; line 9, "Al<sub>2</sub>BD3" should read --Al<sub>2</sub>O<sub>3</sub>--.

Signed and sealed this 12th day of February 1974.

(SEAL)

Attest:

EDWARD M. FLETCHER, JR.  
Attesting Officer

C. MARSHALL DANN  
Commissioner of Patents